

## United States Patent Office

3,663,444

Patented May 16, 1972

Brayton

## 1

3,663,444

WASHING AND CLEANSING AGENTS WITH  
POLYAMIDES HAVING IMPROVED DIRT-  
CARRYING CAPACITYEdmund Schmadel, Mettmann, Germany, assignor to  
Henkel & Cie GmbH, Dusseldorf, GermanyNo Drawing. Filed Apr. 29, 1970, Ser. No. 33,090  
Claims priority, application Germany, May 2, 1969,P 19 22 450.1  
Int. Cl. Cl1d 7/56

U.S. CL. 252—99

6 Claims

## ABSTRACT OF THE DISCLOSURE

A washing and cleansing composition with improved 15 dirt-carrying capacity consisting essentially of (1) a surface-active detergent composition, (2) from 0.1% to 20% by weight, based on the total solids, of a water-soluble or water-dispersible polyamide reaction product of (a) a polyalkyleneimine having an average molecular weight of from 300 to 6000 selected from the group consisting of polyethyleneimines and polypropyleneimines and (b) an organic polycarboxylic acid having from 2 to 10 carbon atoms selected from the group consisting of oxalic acid, alkanedioic acids, alkanetriioic acids, alkenedioic acids, benzenedicarboxylic acids, benzenetricarboxylic acids, cyclohexanedicarboxylic acids, cyclohexanetricarboxylic acids, hydroxyalkanedioic acids, hydroxyalkanetriioic acids, polyoxyalkanedioic acids, polythioalkanedioic acids, polyaminoalkanedioic acids and polyaminoalkanetriioic acids, the molar ratio of alkyleneimine unit to organic polycarboxylic acid being from 100:1 to 5:1, and (3) optionally a non-surface-active builder salt and a compound with an intensified cleaning action.

## THE PRIOR ART

It is known to add to washing and cleaning compositions which contain surface-active compounds, substances which improve the dirt-carrying capacity of the washing liquors. Such substances, subsequently called graying inhibitors, prevent re-absorption of the detached dirt on the cleaned surfaces. These substances are mostly poly-anionic polymers, which are prepared either from natural substances such as cellulose, gelatine or glue or by polymerization of vinyl compounds such as acrylic acid, methacrylic acid, maleic acid and mixtures of these with copolymerizable olefins. The polysulfonates of vinyl polymers have also already been recommended as graying inhibiting additions to washing and cleaning compositions. Of these compounds, however, only carboxymethylcellulose has attained relatively great technical importance, chiefly since it surpasses all known synthetic polymers in its graying-inhibiting action. Carboxymethylcellulose and the said synthetic polymers, however, have the disadvantage that their graying-preventing action is restricted to cellulosic fibers. They are largely inactive in the washing of synthetic fibrous material, chemically altered cellulose or finished cottons. This disadvantage becomes specially noticeable in the case of white textiles from polyester or polyolefin fibers, non-iron cottons and mixed fabrics from the said synthetic fibers and cellulose

## 2

fibers which, in spite of frequent washings, may become gray and consequently of poor appearance.

## OBJECTS OF THE INVENTION

- 5 An object of the present invention is to develop a composition which may not have the aforesaid disadvantages. Another object of the invention is the development of a washing and cleansing composition with improved dirt-carrying capacity consisting of essentially of (1) a surface-active detergent composition, (2) from 0.1% to 20% by weight, based on the total solids, of a water-soluble or water-dispersible polyamide reaction product of (a) a polyalkyleneimine having an average molecular weight of from 300 to 6000 selected from the group consisting of polyethyleneimines and polypropyleneimines and (b) an organic polycarboxylic acid having from 2 to 10 carbon atoms selected from the group consisting of oxalic acid, alkanedioic acids, alkanetriioic acids, alkenedioic acids, benzenedicarboxylic acids, benzenetricarboxylic acids, cyclohexanedicarboxylic acids, cyclohexanetricarboxylic acids, hydroxyalkanedioic acids, hydroxyalkanetriioic acids, polyoxyalkanedioic acids, polythioalkanedioic acids, polyaminoalkanedioic acids and polyaminoalkanetriioic acids, the molar ratio of alkyleneimine unit to organic polycarboxylic acid being from 100:1 to 5:1, and (3) optionally a non-surface-active builder salt and a compound with an intensified cleaning action.

These and other objects of the invention will become more apparent as the description thereof proceeds.

## DESCRIPTION OF THE INVENTION

- 35 The invention provides a washing and cleansing composition with improved dirt-carrying capacity especially for synthetic fibers comprising a surface-active detergent composition, from 0.1% to 20% by weight, based on the total solids, of a water-soluble or water-dispersible polyamide, which is obtained by reaction of a polyethyleneimine or polypropyleneimine of average molecular weight of from 300 to 6000 with a di- and/or tri-carboxylic acid containing 2 to 10 carbon atoms in the molecule and in which the molar ratio of alkyleneimine unit to polycarboxylic acid is from 100:1 to 5:1, and optionally a non-surface-active builder salt and a compound with an intensified cleaning action.

40 The polyamides contained in the new washing compositions are obtainable by known method. It is preferred to use polyethyleneimines as starting substances which have an average molecular weight from 300 to 6000, especially 500 to 3000. Suitable polycarboxylic acids having 2 to 10 carbon atoms are aliphatic or cycloaliphatic, saturated or unsaturated, as well as aromatic, di- and tricarboxylic acids; such as oxalic acid; alkanedioic acids such as malonic, succinic, glutaric, adipic, pimelic, suberic, azelaic, and sebacic acids; alkenedioic acids such as maleic and fumaric acids; alkanetriioic acids such as tricarballylic acid; benzenedicarboxylic acids such as phthalic acid; benzenetricarboxylic acids such as trimesic acid; cyclohexanedicarboxylic acids such as hexahydrophthalic acid; cyclohexanetricarboxylic acids; hydroxyalkanedioic acids such as tartaric acid, hydroxyalkanetriioic acids such as citric acid; and also polycarboxylic acids which contain heteroatoms, especially ether-, thioether- and amine-groups. Examples of such polyvalent

carboxylic acids are polyoxyalkanedioic acids such as diglycolic acid; polythioalkanedioic acids such as thioglycolic acid; polyaminoalkanedioic acids such as iminodiacetic acid and polyaminoalkanetriolic acids such as nitrilotriacetic acid. Mixtures of the above-mentioned carboxylic acids may also be used. The reaction products of polyethyleneimine with dicarboxylic acids are preferred.

The preparation of the polyamides is carried out in known way, for example by heating the mixture of acid and polyalkyleneimine for several hours in vacuo or in the presence of a solvent from which the water formed in the reaction can be azeotropically distilled. Instead of the free di- or tri-carboxylic acids, their derivatives capable of reaction, for example the acid anhydrides, chlorides or bromides, may also be used as starting substances. The amounts of di- or tri-carboxylic acid used per alkyleneimine unit are preferably such that at least one mol of a di- or tri-carboxylic acid is associated with one macromolecule consisting of polyalkyleneimine. The molar ratio of alkyleneimine unit to polyvalent carboxylic acid in the preferred range amounts to 50:1 to 10:1, depending upon the average molecular weight of the polyalkyleneimine.

The polyamides prepared in the manner indicated have a resinous consistency and are soluble or dispersible in water or in solutions of washing compositions. They may still contain minor amounts of unreacted starting substances, which can be removed by extraction with organic solvents and if desired again used in the reaction. Since these compounds do not affect the cleaning properties of the compositions, however, their separation is unnecessary. Owing to the insolubility of the high molecular weight compounds in organic solvents and on account of their content of low-molecular weight fractions, the usual methods of molecular weight determination cannot be used. The degree of polymerization and molecular weight of the final polyamides therefore cannot be given with sufficient accuracy.

In addition to the polyamides, the washing and cleaning compositions according to the invention contain surface-active substances customary in such compositions such as anionic, non-ionic or amphoteric detergent substances. Further, non-surface-active inorganic and/or organic builder salts may be present, as well as compounds which increase the cleaning capacity of the compositions or the degree of whiteness of the treated textiles.

Suitable detergent substances are anionic compounds of the sulfonate or sulfate type, for example alkylbenzene sulfonates; especially n-dodecylbenzenesulfonate, and also olefinsulfonates such as are obtained, for example, by sulfonation of primary or secondary aliphatic monoolefins with gaseous sulfur trioxide and subsequent alkaline or acid hydrolysis. Alkylsulfonates, such as are obtainable from n-alkanes by sulfochlorination or sulfoxidation and subsequent hydrolysis or neutralization, or by addition of bisulfite to olefins, may also be used. In addition,  $\alpha$ -sulfo-fatty acid esters, primary and secondary alkyl sulfates and the sulfates of ethoxylated or propoxylated higher molecular weight alcohols are suitable.

Further compounds of this anionic class which, if desired, may be present in the washing compositions, are the higher molecular weight sulfated partial ethers and partial esters of polyhydric alcohols, such as the alkali metal salts of the monoalkyl ethers or mono-fatty acid esters of glycerinemonosulfuric acid ester or 1,2-dihydroxypropanesulfonic acid respectively. Sulfates of ethoxylated or propoxylated fatty acid amides and alkylphenols and also fatty acid taurides and fatty acid isothiocyanates are also suitable.

Further suitable anionic detergent substances are alkali metal soaps of higher fatty acids of natural or synthetic origin, for example the sodium soaps of coconut, palm kernel or tallow fatty acids. The amphoteric detergent substances may be alkylbetaines and especially alkylsulfobetaines, for example 3-(N,N-dimethyl-N-alkylammonium)-

um)-propane-1-sulfonate and 3-(N,N-dimethyl-N-alkylammonium)-2-hydroxypropane-1-sulfonate.

The anionic detergent substances may be present as the sodium, potassium and ammonium salts or as salts of organic bases, such as mono-, di or tri-ethanolamine. When the said anionic and amphoteric compounds contain an aliphatic hydrocarbon residue, this should preferably be a straight chain and contain 8 to 22 carbon atoms. In compounds with an araliphatic hydrocarbon residue the preferably unbranched alkyl chains contain an average of 6 to 16 carbon atoms.

The most suitable non-ionic surface-active detergent substances are polyglycol ether derivatives of alcohols, fatty acids and alkylphenols which contain 3 to 30 glycol ether groups and 8 to 20 carbon atoms in the hydrocarbon residue. Particularly suitable are polyglycol ether derivatives which contain from 5 to 15 ethylene glycol ether groups and of which the hydrocarbon residues are derived from straight chain primary alcohols having 12 to 18 carbon atoms or from alkylphenols with a straight alkyl chain containing 6 to 14 carbon atoms. By addition of 3 to 15 mols of propylene oxide to a last-named polyethylene glycol ether or by conversion into the acetals, washing substances are obtained which are marked by a particularly low foaming power.

Further suitable non-ionic detergent substances are the water-soluble adducts, containing 20 to 250 ethylene glycol ether groups and 10 to 100 propylene glycol ether groups of polyethylene oxide to polypropylene glycol, ethylenediaminopolypropylene glycol and alkylpolypropylene glycol with 1 to 10 carbon atoms in the alkyl chain. The said compounds usually contain 1 to 5 ethylene glycol units per propylene glycol unit. Non-ionic compounds of the amineoxide and sulfoxide type which, if desired, may also be ethoxylated, are also utilizable.

Suitable mixing components are also inorganic cleaning salts or builders, especially condensed phosphates such as pyrophosphates, triphosphates, tetraphosphates, trimetaphosphates, tetrametaphosphates and more highly condensed phosphates, in the form of the neutral or acid sodium, potassium or ammonium salts. Alkali metal triphosphates and their mixtures with pyrophosphate are preferably used. Further silicates may be used, especially sodium silicate, in which the ratio of  $\text{Na}_2\text{O}:\text{SiO}_2$  amounts to 1:3.5 to 1:1.

The condensed phosphates may also be wholly or partly replaced by organic nitrogen- or phosphorus-containing complex-forming substances with a cleaning action. These compounds include the alkali metal or ammonium salts of nitrilotriacetic acid, ethylenediaminetetraacetic acid, diethylenetriaminopentaacetic acid and the higher homologues of the said aminopolycarboxylic acids. Suitable homologues may be prepared, for example, by polymerization of an ester, amide or nitrile of N-acetic acid azidine and subsequent saponification to the carboxylic acid salts, or by reaction of polyamines with a molecular weight of 500 to 100,000 with salts of chloroacetic acid or bromoacetic acid in an alkaline medium. Further suitable aminopolycarboxylic acids are poly-(N- $\beta$ -propionic acid)-ethyleneimines of average molecular weight from 500 to 200,000 which are obtainable analogously to the N-acetic acid derivatives. Phosphorus-containing complex-forming substances which may be used are the alkali metal and ammonium salts of aminopolypophosphonic acids, especially aminotri-(methyleneephosphonic acid), ethylenediamine-tetra-(methyleneephosphonic acid), 1-hydroxyethane-1,1-diphosphonic acid, methylenediphosphonic acid, ethylenediphosphonic acid and the higher homologues of the said polyphosphonic acids. Mixtures of the aforesaid complex-forming substances may also be used.

Further suitable mixing components are neutral salts such as sodium sulfate and sodium chloride, and substances for regulating the pH such as sodium or potassium bicarbonates, borates and hydroxides, and also acids such as lactic acid and citric acid. The quantity of alka-

line-reacting substances inclusive of the alkali metal silicates and phosphates should be such that the pH of a liquor suitable for coarse washing amounts to 9 to 12 and for fine washing amounts to 6 to 9.

By suitable combination of different surface-active detergent substances and builder salts, increased actions may be obtained in many cases, for example, an improved washing power or a reduced foaming capacity. Such improvements are possible, for example, by combination of anionic with non-ionic and/or amphoteric compounds, by combination of different non-ionic compounds or by mixtures of detergents of the same type which differ in respect to the number of carbon atoms or the number and position of the double bonds or branchings of the chains in the hydrocarbons. Likewise synergistically-acting mixtures of inorganic and organic builder salts may be used or combined with the aforesaid mixtures.

The compositions may contain oxygen-yielding bleaching agents, such as hydrogen peroxide, alkali metal perborates, alkali metal percarbonates, alkali metal perphosphates, urea perhydrate and alkali metal persulfates or active chlorine-containing compounds, such as alkali metal hypochlorites, chlorinated trisodium phosphate and chlorinated cyanuric acid or its alkali metal salts, according to the purpose of use. The pre-compounds may be present in admixture with bleaching activators such as magnesium silicate

Suitable optical brighteners are those of the bis(tri-azinyl)-4,4'-diaminostilbenedisulfonic acid type of the formula:



In the formula R<sub>1</sub> and R<sub>2</sub> signify halogen atoms or alkoxy groups, amino groups or residues of aliphatic, aromatic or heterocyclic, primary or secondary amines, or residues of aminosulfonic acids, while aliphatic residues present in the above groups preferably contain 1 to 4 and especially 2 to 4 carbon atoms, and in the heterocyclic ring systems, five- or six-membered rings are usually concerned. Aniline, anthranilic acid or anilinesulfonic acid residues are preferred as the aromatic amines. Brighteners derived from diaminostilbenesulfonic acid are mostly used as cotton brighteners. The following products derived from the above formula in which R<sub>1</sub> represents the residue  $-\text{NH}-\text{C}_6\text{H}_5$  and R<sub>2</sub> may represent the following residues, are at present on the market:



Some of these brighteners are to be regarded as transitional types to the cotton brighteners as regards their affinity for the fiber, for example, the brightener in which R<sub>2</sub> equals  $-\text{NH}-\text{C}_6\text{H}_5$ . The compound 4,4'-bis-(4-phenyl-vicinal-triazoly-1-2)-stilbenedisulfonic acid - 2,2' also belongs to the cotton brighteners of the diaminostilbenesulfonic acid type.

Further, optical brighteners of the diarylpyrazoline type of the following formula are suitable:



In this formula Ar and Ar' signify aryl residues such as phenyl, diphenyl or naphthyl, which may be substituted by substituents such as hydroxy, alkoxy, hydroxyalkyl, amino, alkylamino, acylamino, carboxyl, sulfonic acid and sulfonamide groups or halogen atoms. It is preferred to use a 1,3-diarylpyrazoline derivative in which the residue Ar represents a p-sulfonamidophenyl group and the residue Ar' represents a p-chlorophenyl group. Besides this, for brightening of other types of fibers, suitable white toners may also be present, for example, those of the type of the naphthothiazolestilbenesulfonates, ethylene-bis - benzimidazoles, ethylene - bis - benzoxazoles, thiophene - bis - benzoxazoles, dialkylaminocoumarins and cyanoanthracene. These brighteners or their mixtures may be present in the compositions in amounts from 0.01 to 1.5% by weight, preferably 0.1 to 1% by weight.

For the purpose of increasing the dirt carrying power, further known graying inhibitors may be added, such as sodium celluloseglycollate or the water-soluble alkali metal salts of polyesters and polyamides or vinyl polymers containing free carboxyl groups. These include the polyesters or polyamides from tri- and tetra-carboxylic acids and dihydric alcohols or diamines, and polymeric acrylic, methacrylic, maleic, fumaric, itaconic, citraconic and aconitic acids as well as the mixed polymerizates of the said unsaturated carboxylic acids or their copolymers with olefins.

Compositions which are intended for use in drum washing machines suitably contain known foam-inhibiting agents, as, for example, saturated fatty acids with 20 to 24 carbon atoms, or their alkali metal soaps, or triazine derivatives which are obtainable by the reaction of 1 mol of cyanuric chloride with 2 to 3 mol of an aliphatic, straight, branched or cyclic chain, primary monoamine or by propoxylation or butoxylation of melamine.

For further improvement of the dirt-loosening properties of the compositions according to the invention, these may also contain enzymes from the class of proteases, lipases and amylases. The enzymes may be of animal and vegetable origin, for example may be obtained from digestive ferments or yeasts such as pepsin, pancreatin, trypsin, papain, catalase and diastase. Enzymic active substances obtained from strains of bacteria or fungi, such as *Bacillus subtilis* and *Streptomyces griseus*, are preferably used which are relatively stable towards alkali, per-compounds and anionic detergent substances and are not appreciably inactivated even at temperatures between 45° and 70° C.

The washing and cleaning compositions may be present in liquid, pasty or solid, for example pulverulent, granulated or lump form. Liquid preparations may contain solvents miscible with water, especially ethanol and isopropanol, and also solution aids such as the alkali metal salts of benzene-, toluene-, xylene-, or ethylbenzene-sulfonic acids. To increase the foaming capacity and to improve the compatibility with the skin, alkylolamides such as fatty acid mono- and di-ethanolamides may be added if desired. Moreover, the mixtures may contain dyestuffs and perfumes, bactericides, substances with a freshening action, and fillers, for example urea.

The preparation of the compositions according to the invention may be effected in the usual way by mixing, granulating or spray drying. If enzymes are used, it is

advisable to mix these with non-ionic detergent substances and possibly perfumes or to disperse them in the melt of a salt containing water of crystallization, for example Glaubers salt, and then to unite these prior mixtures with the remaining powder components. In this way the enzymes are cemented with the other particles of powder so that the mixtures do not tend to form dust or to separate into their components.

The qualitative and quantitative composition of the preparations according to the invention depend largely on their field of use. The content of polyamide from polycarboxylic acid and polyalkyleneimine amounts to 0.1% to 20%, preferably 0.2% to 10% by weight based on total solids. The difference of 80% to 99.9%, preferably 90% to 99.8% by weight is composed of other washing agent components, the quantitative composition of which may correspond to the following scheme (data in percent by weights):

1% to 40% of at least one compound from the class of the anionic, non-anionic and amphoteric surface-active compounds, preferably as utilizable in neutral to alkaline textile washing baths;

10% to 80% of at least one non-surface-active builder salt with a cleaning intensifying action or a complex-forming action;

10% to 50% of a pre-compound, especially sodium perborate, anhydrous or containing water of crystallization or its mixtures with stabilizers and activators;

0.1% to 20% of other assistants and additives.

The surface-active compounds may consist of up to 100%, preferably 5% to 70%, of anionic surface-active compounds of the sulfonate and/or sulfate type; up to 100%, preferably 5% to 40%, of non-ionic surface-active compounds of the polyglycol ether type; and up to 100%, preferably 10% to 50%, of soap.

The builder salts may be composed of up to 100%, preferably 25% to 95%, of alkali metal triphosphates and their mixtures with alkali metal pyrophosphates; up to 100%, preferably 5% to 50%, of an alkali metal salt of a complex-forming substance from the class of polyphosphonic acids, nitrilotriacetic acid, ethylenediaminetetraacetic acid; and up to 100%, preferably 5% to 75% of at least one compound from the class of alkali metal silicates, alkali metal carbonates and alkali metal borates.

The other assistants and additives include, besides the optical brighteners, especially the foam inhibitors which may be present in the compositions according to the invention in a quantity up to 5%, preferably in a quantity of from 0.2% to 3%, and also the enzymes which may be present in a quantity up to 5%, preferably 0.2% to 3%, and the additional graying inhibitors, the amount of which may be up to 5%, preferably 0.2% to 3%.

The present invention will be further described by way of reference to the following specific examples which are not deemed limitative in any respect.

## EXAMPLES

(1) A pulverulent, weakly foaming washing composition:

3% to 15% of a sulfonate detergent from the class of alkylbenzenesulfonates, olefinsulfonates and n-alkane-sulfonates,

0.5% to 5% of an alkylpolyglycol ether ( $C_{12}$ – $C_{18}$ -alkyl) or an alkylphenol polyglycol ether ( $C_8$ – $C_{14}$ -alkyl) with 5 to 10 ethylene glycol ether groups,

0 to 5% of a  $C_{12}$  to  $C_{18}$  soap,

0.2% to 5% of a foam inhibitor from the class of trialkylmelamines and the saturated fatty acids with 20 to 24 carbon atoms, or their alkali metal soaps,

10% to 50% of a condensed alkali metal phosphate from the class of pyro- or tri-polyphosphates,

0.1% to 5% of a polyamide reaction product of polyethyleneimine and di- or tri-carboxylic acids of the invention,

- 1% to 5% of sodium silicate  
10% to 35% of sodium perborate tetrahydrate,  
0 to 5% of enzymes,  
0.05% to 1% of at least one optical brightener from the class of diaminostilbenedisulfonic acid and diarylpyrazoline derivatives.  
0.1% to 30% of an inorganic salt from the class of the alkali metal carbonates, bicarbonates, borates, sulfates and chlorides.  
10 0 to 4% of magnesium silicate,  
0.5% to 3% of sodium celluloseglycolate

## Examples 2-16

15 The graying inhibiting action of the compounds described in the following examples was tested by the known "soil redeposition" method. In this method, 4 small pieces from the fabric to be examined having a total weight of 8.3 gm. together with 1.3 gm. of an artificially soiled cotton yarn are washed three times for 30 minutes each time in a laboratory washing machine. ("Launder-Ometer," registered trademark.) The reflection value is then found with a photometer (Elrepho," registered trademark) using Filter No. 6.

20 25 The combination of dust and skin fat similar to that found in practice used for soiling the cotton yarn consisted of a mixture of kaolin, black iron oxide, soot and synthetic skin fat (comprising  $\frac{1}{3}$  fatty acids,  $\frac{1}{3}$  fat and  $\frac{1}{3}$  hydrocarbons). After soiling, the cotton yarn contained about 11% of pigments and about 2% of skin fat.

30 35 A prior art washing preparation was used of the following composition (in percent by weight):

- 8% of n-dodecylbenzenesulfonate (Na salt)  
3% of oleyl alcohol with 10 ethylene glycol ether groups  
3% of Na soap of saturated  $C_{12}$  to  $C_{22}$  fatty acids  
40% of pentasodium tripolyphosphate  
22% of sodium perborate  
3.5% of sodium silicate ( $Na_2O:SiO_2=1:3.3$ )  
40 45 2.5% of magnesium silicate  
0.2% of Na nitrilotriacetate  
0.3% of an optical brightener

45 50 55 4% of graying inhibitors, as defined below, were added to this preparation and it was made up to 100% with sodium sulfate.

The concentration of the washing composition used was 5 gm. per liter, and the hardness of the water was 10° German hardness. The textile samples consisting of synthetic fabric (polyester fiber) and mixed fabric (polyester fiber with finished cotton and also polypropylene fiber with cotton) were washed at 60° C. and that of finished cotton was washed at 90° C. The proportion by weight of textile material to wash liquor was 1:30. After a washing period of 30 minutes the samples were rinsed four times with distilled water. After three washing treatments the degree of whiteness of the samples was determined photometrically.

For the preparation of the graying inhibitors according to the invention, a solution of the polyethyleneimine of the average molecular weight indicated and polycarboxylic acid, as indicated, in xylene was heated at the boil until 2 mols of water had been azeptropically distilled per mol of polyvalent carboxylic acid. The resin remaining after distilling the solvent was directly utilizable without further treatment.

The average molecular weight of the polyethyleneimine used, the polycarboxylic acid used, and the molar ratio (mols of ethyleneimine units per mol of di- or tri-carboxylic acid) are given in the following Table I, as well as the remission values of the washed textiles. For comparison, washing experiments were carried out without use of a graying inhibitor and with use of sodium celluloseglycolate respectively. The results show a distinct superiority of the compositions according to the invention.

TABLE I

| Example | Graying inhibitor                                  |                   | Remission of values of the textile samples |           |                                |                           |                 |
|---------|----------------------------------------------------|-------------------|--------------------------------------------|-----------|--------------------------------|---------------------------|-----------------|
|         | Average molecular weight of the polyethyl-eneimine | Dicarboxylic acid | Molar ratio                                | Polyester | Polyester with finished cotton | Polypropylene with cotton | Finished cotton |
| 2.      | 600                                                | Oxalic acid       | 14:1                                       | 58.9      | 65.7                           | 56.7                      | 80.1            |
| 3.      | 1,200                                              | do                | 28:1                                       | 60.9      | 65.3                           | 59.8                      | 80.5            |
| 4.      | 1,800                                              | do                | 42:1                                       | 58.7      | 60.5                           | 54.1                      | 81.7            |
| 5.      | 600                                                | Succinic acid     | 14:1                                       | 58.9      | 66.6                           | 60.2                      | 80.3            |
| 6.      | 1,200                                              | do                | 28:1                                       | 58.0      | 57.0                           | 53.8                      | 78.6            |
| 7.      | 1,800                                              | do                | 42:1                                       | 58.6      | 61.4                           | 58.3                      | 82.6            |
| 8.      | 600                                                | Adipic acid       | 14:1                                       | 58.2      | 74.7                           | 59.9                      | 79.4            |
| 9.      | 1,200                                              | do                | 28:1                                       | 59.3      | 76.3                           | 63.0                      | 75.2            |
| 10.     | 1,800                                              | do                | 42:1                                       | 60.3      | 63.9                           | 62.4                      | 82.5            |
| 11.     | 600                                                | Terephthalic acid | 14:1                                       | 60.8      | 66.4                           | 59.4                      | 80.5            |
| 12.     | 1,200                                              | do                | 28:1                                       | 57.2      | 61.1                           | 57.6                      | 77.6            |
| 13.     | 1,800                                              | do                | 42:1                                       | 62.1      | 63.9                           | 58.9                      | 82.5            |
| 14.     | 600                                                | Citric acid       | 14:1                                       | 57.6      | 75.3                           | 48.7                      | 81.4            |
| 15.     | 1,200                                              | do                | 28:1                                       | 58.7      | 75.6                           | 50.2                      | 82.0            |
| 16.     | 1,800                                              | do                | 42:1                                       | 5.97      | 74.3                           | 50.5                      | 81.8            |
| A.      | Without graying inhibitor                          |                   |                                            | 38.7      | 53.1                           | 35.6                      | 60.7            |
| B.      | Sodium celluloseglycolate                          |                   |                                            | 38.9      | 53.4                           | 36.0                      | 60.5            |

The preceding specific embodiments are illustrative of 25 the practice of the invention. It is to be understood, however, that other expedients known to those skilled in the art, or described herein, may be employed without departing from the spirit of the invention or the scope of the appended claims.

I claim:

1. A washing and cleansing composition with improved dirt-carrying capacity consisting essentially of
  - (1) from 80% to 99.9% by weight of a detergent composition consisting essentially of
    - (a) from 1% to 40% of at least one surface-active compound utilizable in neutral to alkaline textile washing baths selected from the group consisting of anionic surface-active compounds, non-ionic surface-active compounds, amphoteric surface-active compounds, and mixtures thereof,
    - (b) from 10% to 80% of at least one non-surface-active builder salt which is an alkali metal salt of an acid selected from the group consisting of tripolyphosphoric acid, pyrophosphoric acid, polyphosphonic acids, nitrilotriacetic acid, ethylenediaminetetraacetic acid, silicic acid, carbonic acid and boric acid,
    - (c) from 10% to 50% of a bleaching compound selected from the group consisting of per-compounds and mixtures of per-compounds with stabilizers and activators,
    - (d) from 0.1% to 20% of other customary washing composition assistants and additives including at least one of from 0.2% to 5% enzymes, from 0.2% to 5% of customary graying inhibitors, and from 0.01% to 1.5% of optical brighteners and,
  - (2) from 0.1% to 20% by weight, based on the total solids, of a water-soluble or water-dispersible polyamide reaction product of (a) a polyalkyleneimine having an average molecular weight of from 300 to 6000 selected from the group consisting of polyethylenimines and polypropyleneimines and (b) an organic polycarboxylic acid having from 2 to 10 carbon atoms selected from the group consisting of oxalic acid, alkanedioic acids, alkanetriioic acids, alkenedioic acids, benzenedicarboxylic acids, benzenetricarboxylic acids, cyclohexanedicarboxylic acids, cyclohexanetricarboxylic acids, hydroxyalkanedioic acids, hydroxyalkanetriioic acids, polyoxy-

alkanedioic acids, polythioalkanedioic acids, polyaminoalkanedioic acids and polyaminoalkanetriioic acids, the molar ratio of alkyleneimine unit to organic polycarboxylic acid being from 100:1 to 5:1.

2. The washing and cleansing composition of claim 1

30 wherein said surface-active compound of component (1) (a) is selected from the group consisting of sulfonates, sulfates, soap and polyglycol ethers.

3. The washing and cleansing composition of claim 2 wherein said surface-active compound of component (1)

35 (a) consists essentially of (i) from 25% to 75% of said sulfonates and sulfates, (ii) from 5% to 40% of said polyglycol ethers, and (iii) from 10% to 50% of said soaps.

4. The washing and cleansing composition of claim 1

40 wherein said non-surface-active builder salts of component (1)(b) consists essentially of (i) from 25% to 95% of said alkali metal tripolyphosphates and pyrophosphates, (ii) from 5% to 50% of said alkali metal salts of said polyphosphonic acids, said nitrilotriacetic acid 45 and said ethylenediaminetetraacetic acid, and (iii) from 5% to 75% of said alkali metal silicates, carbonates and borates.

5. The washing and cleansing composition of claim 1 wherein said bleaching compound of component (1)(c)

50 is selected from the group consisting of anhydrous sodium perborate and water-of-crystallization-containing sodium perborate.

6. The washing and cleansing composition of claim 1 wherein said other customary washing composition as-

55 sistants and additives of component (1)(d) include from 0.2% to 5% of at least one foam inhibitor selected from the group consisting of saturated fatty acids containing 20 to 22 carbon atoms and their alkali metal soaps, substituted triazines obtained by reaction of 1 mol of cyanuric 60 chloride with 2 to 3 mols of a primary monoamine and propoxylation and butoxylation products of melamine.

#### References Cited

#### UNITED STATES PATENTS

65 3,262,791 7/1966 Dickson et al. 252—137 UX  
3,563,902 2/1971 Schmadel et al. 252—99 X

MAYER WEINBLATT, Primary Examiner

70 U.S. Cl. X.R.

252—525, 544, DIG 2, DIG 15; 260—78 TF, 78 A, 2 EN